

C. J. A. DALZIEL.  
PROCESS OFrecovering COPPER FROM ITS ORES.  
APPLICATION FILED SEPT. 24, 1918.

1,341,786.

Patented June 1, 1920.



Witnesses  
*Frank C. Clegg*

By his Attorneys

Inventor  
C. J. A. Dalziel  
*Baldwin Wright*

# UNITED STATES PATENT OFFICE.

CHARLES JOSEPH ALBERT DALZIEL, OF LONDON, ENGLAND.

## PROCESS OF RECOVERING COPPER FROM ITS ORES.

1,341,786.

Specification of Letters Patent. Patented June 1, 1920.

Application filed September 24, 1918. Serial No. 255,469.

*To all whom it may concern:*

Be it known that I, CHARLES JOSEPH ALBERT DALZIEL, a subject of the King of Great Britain, whose residence is in London, England, have invented certain new and useful Improvements in Processes of Recovering Copper from Its Ores, of which the following is a specification.

According to this invention copper is extracted and precipitated directly from a pulped copper ore by a single continuous operation without filtration. According to this invention the copper ore is supplied to one or more preparatory vessels through a chute or chutes which is provided with suitable means for controlling the supply of ore to the vessel and a dilute acid solution is supplied to the preparatory vessel through a pipe or conduit provided with suitable means for regulating the supply of the solution to said vessel.

The preparatory vessels are identical in construction and equipment. Either one or both of the preparatory vessels may be used and the continuous operation of the process need not be affected by the failure for any reason of either of said vessels as both being identical in construction either one can carry on the process independently of the other if necessary.

The solution and the finely crushed copper ore together form a bulk of acid pulp containing copper ore in a liquid. The pulp is agitated and aerated in the preparatory vessel or vessels by compressed air injected into the same for purpose of keeping the ore in suspension in the solution. The ore thus treated is led to the first of a series of electrolytic vessels where it is agitated and aerated by compressed air, and an electric current is passed from an insoluble anode through the pulp to a cathode upon which the copper is deposited by the action of the electric current.

The pulp is then led to the second of the series of electrolytic vessels similarly equipped with electrodes and with means for agitating and aerating the pulp and is then led from the second to the third electrolytic vessel in the series and is then led through the remainder of the series of electrolytic

vessels, which series may consist of any number of vessels or cells equipped with electrodes and with means for agitating and aerating the pulp by compressed air. The 55 number of electrolytic vessels will depend upon the length of time required to deposit the copper contained in the pulp upon the cathodes.

As the pulp is led from the preparatory vessel to the electrolytic vessels or cells, fresh ore and acid solution is added to the preparatory vessel to provide a continuous supply of acid pulp to take the place of the pulp which is drawn off from the last electrolytic vessels and which has become depleted of its copper content by electrolysis.

By regulating the flow of ore and of solution into the preparatory vessels and correspondingly regulating the flow of depleted pulp from the last of the series of electrolytic vessels a continuous supply of freshly charged pulp of approximately uniform strength in copper is delivered to the electrolytic vessels, thus enabling a uniform 75 strength of electric current to be used and insuring a continuous cycle of operations which need only be interrupted for the purpose of carrying out repairs or replacements should such become necessary.

Furthermore, as the copper is recovered direct from the pulp, the ore being kept in suspension through agitation and aeration by compressed air, the process eliminates all filtering and its attendant evils.

The number of electrolytic cells employed is sufficient relatively to the rate of flow of the pulped ore to substantially exhaust the copper content of the ore by the time the latter is discharged from the last cell.

The ore may be roasted or not, depending upon the character of the particular ore under treatment. Thus with sulfid ores it is preferable to roast the ore at the commencement of the operation, thereby converting a large part of the copper content of the ore into sulfate, during which operation a part of the copper will ordinarily be converted into oxid.

The process may be conveniently carried out in an apparatus of the kind illustrated in the accompanying drawings in which:

Figure 1 is a diagrammatic view of a suitable apparatus for practising the process.

Fig. 2 shows on a larger scale a vertical section of one of the electrolytic vats or cells.

Ore is fed into the preparatory vessels 1 and 1<sup>A</sup> through chutes 2 in regulated quantities. Valves or gates 2<sup>a</sup>, as indicated, regulate the flow of the ore. An acid leach solution is fed to each preparatory vessel from a tank 3 through pipes 4 each provided with a valve 4<sup>a</sup>, the amount of solution fed being such as to produce a thin flowable pulp in the preparatory vessels. I prefer to introduce the ore and the solution simultaneously so that there will be more or less agitation produced as they enter the vessels.

In order to produce a complete suspension of the ore in the preparatory vessels a blast of air is introduced through a perforated pipe 5 at the bottom of each vessel. The air thus introduced produces aeration and agitation of the pulp so that a more or less homogeneous flowable pulp is produced and the ore particles are held at all times in suspension. The air thus introduced also serves to some extent to aid solution of the copper contained in the suspended ore.

The pulp being thus thoroughly aerated and agitated is allowed to flow off through the pipes 6 having valves *a* into the first of a series of electrolytic cells or vats 7, 8, etc., to 9, these cells being provided with insoluble anodes and cathodes and with an air blast 10 located at the bottom of each vessel for the purpose of maintaining the ore in suspension therein and for agitating and aerating it. The liquid flows from cell to cell through suitable overflow connections 11 and the exhausted ore is drawn off through a pipe 12 provided with a regulating valve 12<sup>a</sup>. Suitable electrical connections are provided at 13 and 14 for the anodes and cathodes.

Assuming the liquid in tank 3 to contain some sulfuric acid, this acid will dissolve (in the preparatory vessels) a certain amount of the copper in the ore under treatment which, as previously stated, may be roasted if desired. It is not intended to employ an amount of sulfuric acid capable of dissolving the entire copper content of the ore and in practice only a small quantity of sulfuric acid is employed, since the electrolysis of the liquor in each of the electrolytic cells will regenerate a portion of the sulfuric acid, which portion being regenerated in a substantially nascent state reacts at once with more of the copper contained in the ore.

In each of the cells 7, 8, etc., to 9, insoluble anodes 15 are suspended and are associated with cathodes 16.

The anodes are connected to a suitable

support 17, connected to the positive wire 65 of a suitable generator or other source of electricity and the cathodes are properly connected to the negative wire 14 of the circuit.

It will be observed that I do not at any stage of the operation subject the pulped ore to filtration, which operation is expensive not only in apparatus employed but in the attendance required. It also will be observed that I do not, at any stage of the process, heat or boil the liquor, and the entire operation taking place in the apparatus illustrated is conveniently conducted at ordinary atmospheric temperature. I thereby avoid the expense incident to heating the liquors, and to maintaining said liquor in a heated state. The number of electrolytic cells depends upon the speed of flow desired and the time required to deposit substantially the entire content of copper contained in the ore.

In practice it is advisable after starting the operation to introduce continuously in regulated amounts the finely crushed ore through the chutes 2 and regulated amounts 90 of liquid from the tank 3, thereby maintaining a full supply of the ore and liquid in the preparatory vessels. In this way the overflow through the pipe 6 and the passage of the liquid through the pipes 11 and discharge pipe 12 is made continuous and requires little service from an attendant.

As the drawings indicate, I preferably employ two preparatory vessels 1 and 1<sup>A</sup> and the copper ore is supplied to both of these vessels, which are identical in construction and equipment. The ore is supplied through two chutes 2, each of which is provided with means for controlling the supply to the vessel, and a dilute acid solution is supplied to both vessels through pipes or conduits 4, each provided with suitable means 4<sup>a</sup> for regulating the supply of the solution to said vessels. Either one or both of the preparatory vessels may be used and 110 the continuous operation of the process need not be affected by the failure for any reason of either of the preparatory vessels. Either one can carry on the process independently of the other if necessary.

I claim as my invention:

1. The herein described process of extracting copper from its ores which consists in supplying to a preparatory vessel finely crushed ore and an acid solution, in such proportions as to produce a flowable pulp, forming the said ore and solution into a flowable pulp by aeration-agitation in said vessel, passing the pulp of liquor and ore once only through a series of electrolytic 125 cells separate from said preparatory vessel, while preventing sedimentation in said cells by introducing a blast of air at the lower

part of each of said cells, and continuously discharging the substantially barren pulp from the last of said cells.

2. The herein described process of extracting copper from its ores, which comprises supplying to a preparatory vessel crushed ore substantially free from sulfid, and an acid solution containing a fraction only of the amount of acid which would be chemically equivalent to the copper content of the said ore, in such proportions as to form a readily flowable pulp, forming the said ore and solution into a flowable pulp solely by aeration-agitation in said vessel, passing the pulp of liquor and ore once only through a series of electrolytic cells separate from said preparatory vessel, while preventing sedimentation in said cells, and continuously discharging the substantially barren pulp from the last of said cells.

3. The herein described process of extracting copper from its ores which consists in supplying to a preparatory vessel, finely crushed ore and an acid solution containing a fraction only of the amount of acid which would be chemically equivalent to the copper content of the said ore, in such proportions as to produce a flowable pulp, forming the said ore and solution into a flowable pulp by aeration-agitation in said vessel, passing the pulp of liquor and ore once only through a series of electrolytic cells separate from said preparatory vessel, while preventing sedimentation in said cells, and continuously discharging the substantially barren pulp from the last of said cells, all of said operations being conducted at normal atmospheric temperatures.

4. A process of extracting copper from copper ore, which comprises pulping finely divided ore with an acid leaching solution by aeration-agitation only, said solution containing a fraction only of that amount of acid which would be necessary to dissolve the entire copper content of the ore, and without filtration of said pulp, causing the same to flow through a series of electrolytic cells until the copper content of the pulp is

commercially exhausted while agitating the ore pulp as it passes through said cells, to prevent sedimentation.

5. A process of extracting copper from sulfid ores containing copper which comprises first subjecting the ore to a sulfatizing roast, whereby the copper is converted principally into sulfate and oxid, subjecting the finely divided roasted ore and an acid leaching solution to sufficient agitation to produce a readily flowable thin pulp, passing such pulp once only through a series of electrolytic cells until the copper content of the pulp is commercially exhausted and discharging the pulp from the system.

6. The herein described process of extracting copper from its ores which consists in supplying to a preparatory vessel finely crushed ore and an acid solution, in such proportions as to produce a flowable pulp, such solution containing materially less acid than would correspond to the amount of copper in the said ore, forming the said ore and solution into a flowable pulp by aeration-agitation in said vessel, passing the pulp of liquor and ore once only through a series of electrolytic cells separate from said preparatory vessel, while preventing sedimentation in said cells, and continuously discharging the substantially barren pulp from the last of said cells.

7. A process of treating oxidized copper ores which comprises continuously subjecting the said ore, in a finely divided state, in a leaching solution, at about atmospheric temperature, to agitation produced solely by a blast of air of sufficient intensity and for a sufficient length of time to produce a readily flowable thin pulp, and continuously passing such pulp through a series of electrolytic cells, while agitating the pulp solely by an air blast sufficient to prevent any such amount of sedimentation in the cells as would substantially obstruct the same.

In testimony whereof I have hereunto subscribed my name.

CHARLES JOSEPH ALBERT DALZIEL.